

C. T. HOLCROFT,  
PROCESS OF ANNEALING MALLEABLE CAST IRON.  
APPLICATION FILED JAN. 20, 1921.

1,422,710.

Patented July 11, 1922.

3 SHEETS—SHEET 1.



C. T. HOLCROFT,  
PROCESS OF ANNEALING MALLEABLE CAST IRON,  
APPLICATION FILED JAN. 20, 1921.

1,422,710.

Patented July 11, 1922.

3 SHEETS—SHEET 2.

*Fig. 3.*



*Fig. 4.*



*Fig. 5.*



Inventor

Charles T. Holcroft,

*By* *Charles T. Holcroft*  
Attorneys

C. T. HOLCROFT,  
PROCESS OF ANNEALING MALLEABLE CAST IRON.  
APPLICATION FILED JAN. 20, 1921.

1,422,710.

Patented July 11, 1922.

3 SHEETS—SHEET 3.



# UNITED STATES PATENT OFFICE.

CHARLES T. HOLCROFT, OF DETROIT, MICHIGAN.

## PROCESS OF ANNEALING MALLEABLE CAST IRON.

1,422,710.

Specification of Letters Patent.

Patented July 11, 1922.

Application filed January 20, 1921. Serial No. 438,608.

To all whom it may concern:

Be it known that I, CHARLES T. HOLCROFT, a citizen of the United States of America, residing at Detroit, in the county of Wayne 5 and State of Michigan, have invented certain new and useful Improvements in Processes of Annealing Malleable Cast Iron, of which the following is a specification, reference being had therein to the accompanying 10 drawings.

This invention relates to a process of annealing malleable cast iron.

It has for its object the production of 15 castings in which the graphitizing of the carbon is conducted at a much more rapid rate than is customary in the prior art.

A further object of my invention is to obviate the necessity for packing the castings in pots or boxes.

20 By the use of a preferred form of apparatus, I accomplish the further result of passing the castings continuously through the annealing process under predetermined conditions of temperature during each stage 25 of the annealing operation. I accomplish the above and other objects by the use of a furnace in which the heat is applied directly to the castings by means of an un-protected electric heating element, the fur-

30 nace being so constructed that access of oxygen during the annealing operation may be prevented. The castings entering at one end of the furnace in the preferred form of apparatus are made to progress continu- 35 ously past a series of heating elements, the temperature of which is so regulated that the castings will first be raised in temperature at a substantially uniform rate per hour to the predetermined annealing tem- 40 perature. They will be maintained at annealing heat for a predetermined period, and in their further progress through the ap- 45 paratus, the heating conditions will be regu- lated so that the castings will be lowered in temperature at a predetermined rate per hour until the critical point of temperature has been passed, after which the castings 50 may be immediately removed from the fur- nace and cooled rapidly down to the atmos- pheric temperature.

By this method the expense of providing cast iron or steel annealing pots or boxes is rendered unnecessary. The time hitherto

consumed in packing the castings before heating as well as the time hitherto lost in 55 waiting for the packed castings to cool down to a temperature at which they could be handled is saved.

By the usual methods, annealing is ac- 60 complished in two ways. In the first, the castings are placed in containers such as pots or boxes and packed with iron oxide, either as hematite or as mill scale; or in some cases where a large amount of small work is being carried on, the small castings 65 are used as a packing. Slag, sand, clay, and lime, or substantially any refractory mate- rial may be used instead of the iron oxide.

The pots or containers are then placed into 70 a large furnace and the heat is applied di- rectly. The boxes are arranged in such a way that the flames may play around them as completely as possible. The flames come in from the top and pass out at the bottom along the sides. The fuel may be coke, coal, 75 oil, or gas, gas being preferred as more read- ily controlled for uniformity of heating. The pots act not only as containers to hold the castings but also to prevent oxidization. The pots become oxidized and scale off, or 80 crack and become unfit for use after a few operations.

Where iron oxide is used as a packing, a portion of the carbon in the castings unites with the oxygen of the oxide and when a 85 casting is broken there is a white skin layer. If the composition of the metal and the con- ditions were correct, a black heart casting 90 may be produced by a proper anneal but, should the temperature of annealing be too high, or be continued too long, the black heart fracture may change to a steely frac- ture, showing an iron in which the precipi- 95 tated carbon has returned to the combined form. If the annealed castings are cooled too fast after the anneal, or if the black heart castings, after being successfully made are reheated and hammered, or reheated and quenched in water, the black heart fracture will change to steely. Graphite should nor- 100 mally separate from irons high in carbon during and shortly after solidification. The rapid cooling in casting prevents this sepa- ration. Reheating to a point below fusion causes a slow readjustment of conditions by 105 the occurrence of the reaction that was pre-

viously suppressed. If however, the annealing is continued too long, the carbon precipitated from the solid solution enters into combination with the iron to form the carbide. As the metal cools, this carbide separates and we get the steely fracture. If we depend for annealing on the oxidation of carbon, we get white heart castings; if we graphitize the cementite, we get the black heart castings.

It takes about six days for the ordinary American annealing operation including heating up and cooling down. Sometimes this can be shortened a little by decreasing the time of the full annealing heating, or by cooling rapidly, or drawing the containers out of the oven and dumping them while the castings are still at a red heat. This does not give good quality of castings. In a relatively rapid cooling there is no time for the graphitization of cementite and much less is there time for graphitization of pearlitic cementite. A very slow cooling affords time for the graphitization not only of the cementite but also of any pearlite which may be present. If the time of the full annealing temperature is reduced, the annealing temperature must be made higher, but the higher heat reduces the strength and ductility of the castings. In prolonged annealing the temper carbon tends to form larger flakes and the metal may become oxidized between the grains, i. e., "burnt."

The second method of annealing is by the use of a muffle type furnace. The castings are piled inside the muffle and the heat is radiated through the muffle. The purpose of the muffle is to eliminate oxidization. The time cycle required, owing to the large mass, is from five to ten days. The average charge is approximately twenty tons. The method of heating both types of furnaces is either by coal hand-fired, or stoker-fired, by coke, by oil, or by gas, any of these requiring the attention of a man to regulate the temperature at various intervals during the process. This, of course, makes a very uncertain element, as it is impossible to maintain close regulation of temperature on large furnaces, using the above mentioned fuels.

In the drawings;

Figure 1 is a horizontal section of the preferred form of furnace employed in carrying out my invention, parts being broken away; Fig. 2 is a central vertical longitudinal section of the furnace, corresponding parts being broken away;

Fig. 3 is a transverse vertical section on the line III—III of Fig. 1;

Fig. 4 is a vertical section on the line IV—IV of Fig. 1;

Fig. 5 is a vertical section on the line V—V of Fig. 1;

Figs. 6, 7 and 8 are, respectively, a horizontal section, a longitudinal vertical sec-

tion and a transverse vertical section of another type of furnace which may be used in carrying out a modified form of my invention.

Referring to Figs. 1 to 5, I have shown an annealing chamber or leir of the continuous type consisting of three sections, A, B and C, in which an outer metallic casing 1, preferably of steel surrounds all three sections of the furnace. The sections A and B are preferably formed of an inner portion 2 of fire-brick or other suitable heat resisting material and outer portions 3 of heat insulating brick. In the section C, the outer layer of insulating brick is omitted, the wall consisting merely of a layer of fire-brick surrounded by the steel casing. A recess 4 extends along each side of the section A and within these recesses are mounted heating elements 5 consisting of a series of ribbon-type resistances fully exposed, each section being controlled by any suitable automatic temperature regulating means. Additional resistance elements 6 are arranged just beneath the ceiling of the chamber, these being controlled by the same automatic regulating devices.

It will be apparent that four factors may be varied to suit varying conditions. First, the quantity of current may be made to vary either in the entire system or in any section of the resistance elements, since the sections will usually be arranged for independent control. Second, the voltage may also be varied without change in quantity of current. Third, the time during which a casting is exposed to any predetermined temperature is also capable of regulation either by varying the speed of the conveyor, or by varying the length of the chamber. And fourth, the number of resistance elements in use may be made greater or less at any portion of the period of travel of the material. Since the specific construction of the regulating and indicating mechanisms forms no part of the present invention, it has not been deemed necessary to illustrate any of the many types which may be used, but the procedure will be similar in each case. Each different composition of material will require a temperature range and a period of time during which each portion of the annealing operation is accomplished, which will be dependent upon the formula. To determine the time and temperature factors a sample lot of the castings will be exposed in a furnace having a recording pyrometer system.

As the temperature rises, a point will be reached at which a continuous expenditure of energy in heating will not be accompanied by a corresponding rising in temperature. This indicates that a temperature has been reached at which some chemical change is occurring. Either the voltage or the quantity of current or the number of elements in

- use will be increased to cause a further rise of say 200° in order to hasten the action. In most cases, under these conditions, at least ninety per cent of the chemical change will have occurred within less than an hour. From this point, the temperature may be steadily reduced and the remainder of the annealing will occur while the temperature falls.
- Having made the test and noting the indications of the pyrometer record, it will then be easy to construct a controlling mechanism, the nature of which will be dependent upon the type of apparatus used, which will control the quantity of current, its voltage, the number of elements in use, or the rate of speed of the conveyor for any given length of furnace, so that the conditions determined during the preliminary test may be mechanically repeated by the automatic controlling mechanism. An endless conveyor 7 supported upon wheels 8 is used to carry the articles to be annealed lengthwise of the annealing chamber. The wheels 8 roll upon rails 9 carried upon a supporting frame work 10, which also forms the support for the entire annealing chamber. As shown in Figs. 3 to 5, the chamber is preferably surrounded by a pit 11 having cement walls and floor, sufficient space being provided between the pit walls and the sides of the chamber to permit workmen to have ready access to the space beneath the annealing chamber. Secured to the under portion of the supports 10 are flanged tracks 12, upon which the endless conveyor is supported on its return journey beneath the annealing chamber. Upon the sides of the sections of the endless conveyor are flanges 13, which extend into troughs 14 containing sand or other refractory material for the purpose of maintaining a substantially air tight seal which not only prevents the passage of air but also acts as an insulating member to prevent loss of heat.
- The movement of the endless conveyor 7 may be continuous or intermittent. The material enters at the left hand end in Figs. 1 and 2 and the temperature is raised in section A at the rate of about 160° F. per hour until a temperature of about 1650° F. is reached, this, of course, requiring about ten hours. The material will be held at the temperature of about 1650° F. for a period of twelve hours to permit substantial completion of the chemical change of the combined carbon in the cementite of the castings into graphite. More than ninety per cent of the entire change will occur at this temperature. The temperature will then be reduced at the rate of 12½° per hour for about twenty-three hours, or to a point between 1360 and 1365° F. and then will be reduced at the rate of approximately 25° per hour for about fifteen hours. The castings will now be reduced to a temperature of about 1,000° F. and the complete cycle of malleabilization will have been completed. During this lowering of temperature, the chemical changes that were most rapid at the upper temperature continue to the practical limit desired. The castings may then be cooled as rapidly as possible. This makes the total time required for the process about sixty hour as compared with the present practice of about one-hundred twenty hours or more.
- The above figures represent the treatment given to malleable iron of a certain specification which represents the longest average cycle required. The complete operation has been done in forty-four hours. The time and temperature factors are entirely dependent upon the chemical analysis of the material.
- While the castings are traveling through the sections B of the annealing chamber, comparatively little heat will be lost because of the presence of the heat insulating brick 3, but in the section C, the rate of cooling will be more rapid because the layer of brick 3 has been omitted and there is only a layer of firebrick 2 inside the metallic casing 1. Since the cooling is divided into two portions of unequal rate, the relative lengths of the periods being substantially the same regardless of the composition of the material, the relative lengths of the two sections B and C as well as the relative rate in which cooling will occur in each section may be predetermined, the time during which the material will remain in the two sections being dependent upon the rate of speed of the endless conveyor.
- Uniformity of results requires uniformity of action, and thus it is necessary that too great differences of temperature between different portions of the material shall be avoided. Since the rate at which heat is conducted by the metal is a function of the composition, the rate at which the initial heating may proceed will depend upon the differences in temperature attained by the least exposed or most remote portion as compared with the portion receiving the greatest heat. So long as too great differences in temperature are avoided, the heating may be made to proceed very rapidly. Thus light or thin castings may be heated more rapidly than thick ones.
- By the use of an air tight metallic casing, no air can reach the interior of the annealing chamber through the side walls, and by the use of electric heating elements no gases are introduced during the heating operation. Any oxygen which enters as the castings are introduced into the chamber may be caused to combine with oil, coke or wood within the chamber so that during the annealing cycle, a neutral or non-oxidizing atmosphere is maintained.

In the modified form of annealing chamber shown in Figs. 6, 7 and 8, the material is loaded upon a car 15 running on a track 16. The car is placed in a chamber 17 similar to 5 the section A of the continuous type of chamber illustrated in Fig. 1. This chamber has an outer casing 1, an inner layer of fire-brick and an intermediate insulating layer in every respect identical with the corresponding structure of the continuous type 10 annealing chamber. The air seal 13—14 is of the same type and the resistance ribbons 5 have an automatic controlling mechanism of the same general type as is provided for 15 the heating elements in the first form of an annealing chamber. With an annealing chamber of this modified type, the variations in temperature will occur through the action of the automatic control mechanism while 20 the castings remain stationary instead of traveling continuously or intermittently as in the previous structure. The same gradual increase of temperature, the maintenance of the annealing temperature for a predetermined 25 period and the gradual decrease in temperature may be accomplished in this form of chamber just as in the other, the only essential difference being the much smaller capacity of the modified form.

30 In the annealing furnaces of the type now in general use, after the annealing operation has been completed, the heavy door of fire-brick which closes one end of the furnace is removed and during a period of about forty- 35 eight hours, the temperature within the furnace is so great that workmen cannot enter to remove the pots containing the castings. Besides this loss of time and also the loss of the heat latent in the furnace walls, after a 40 new batch of material has been set in place in the furnace, a considerable time is required, as well as the expenditure of a considerable amount of fuel, to raise the furnace to the temperature it had when the previous 45 annealing operation was completed.

By my process, I avoid the loss of heat, both at the beginning and at the end of the annealing operation, for, in the continuous type, the furnace never need be allowed to 50 cool, and in the alternative form of furnace shown in Figs. 6, 7 and 8, the material on the car 15 may be withdrawn from the furnace at the end of the annealing operation and a new batch of material already loaded 55 upon another car may be placed immediately in the hot furnace.

A further saving is effected because in the present process where no packing is necessary all of the labor hitherto employed 60 in loading the pots and packing them is done away with, and this in commercial practice represents a very considerable part of the cost of the annealing operation. Also the cost of the pots as well as the labor of handling them is saved.

It has been found that my present process of annealing malleable castings has improved the quality of the surface of the iron probably because of the fact that, by eliminating packing, we prevent the possibility of the 70 absorption by the casting of carbon that may be contained in the packing materials. The structure of the material is more uniform and does not have the high carbon skin commonly found in castings annealed in mill 75 scale or the other mixtures used for packing.

I claim:

1. The method of annealing malleable iron castings which consists in exposing the material to temperatures variable in a definite progression, such progression being effective to raise the temperature of the material at a rate proportionate to the thermal conductivity to a predetermined point of reaction, to maintain reaction temperature for 85 a predetermined time, and then to lower the temperature to a point below which rapid cooling will not injuriously affect the material.

2. The method of annealing malleable iron 90 castings which consists in exposing the material in an atmosphere substantially devoid of oxygen to heat for a period during which the temperature of the castings rises to a degree above that at which conversion of 95 combined carbon into graphite begins and thereafter so controlling the temperature that the desired chemical change will occur before the material has lost sufficient heat to render further chemical change negligible. 100

3. The method of annealing malleable iron castings which consists in exposing the material for a predetermined length of time in an atmosphere substantially devoid of oxygen to heat, the temperature first being raised 105 at a rate proportionate to the thermal conductivity of the material to a higher point than that at which the chemical changes begin, the temperature being maintained at this high point until a predetermined amount 110 of chemical change has occurred, and the temperature then being gradually lowered at a rate such that the desired amount of chemical change shall have been completed by the time the temperature has reached a 115 point at which further chemical change is negligible.

4. The method of annealing malleable iron castings which consists in exposing the material in an atmosphere substantially devoid 120 of oxygen to heat, the temperature during the first period of exposure being increased at a rate substantially proportionate to the thermal conductivity of the material to a point higher than that at which the desired 125 chemical changes begin, the temperature during the next period being maintained substantially uniform at the high point reached at the end of the first period until a predetermined amount of chemical change has oc- 130

curred, and the temperature during a third period being lowered first slowly while further chemical change proceeds and then more rapidly as the rate of chemical change decreases, to a point at which the desirable qualities of the material will not be injuriously affected by rapid cooling.

5. The method of operating an electrically heated furnace for annealing malleable iron castings, which consists in controlling the electrical conditions of some of the heating elements so that the temperature will rise at a predetermined rate to a degree above that at which conversion of combined carbon into graphite begins and thereafter controlling the electrical conditions of some of the heating elements so that the temperature may be maintained substantially uniform for a predetermined period and then controlling the electrical conditions of some of the heating elements to cause a gradual decline in temperature for a predetermined period.

6. The method of operating an electrically heated furnace provided with means whereby an atmosphere substantially devoid of oxygen may be maintained therein for annealing malleable iron castings, which consists in controlling the electrical conditions of some of the heating elements so that the temperature will rise at a predetermined rate to a point above that at which conversion of combined carbon into graphite begins and thereafter controlling the electrical conditions of some of the heating elements so that the temperature may be maintained substantially uniform for a predetermined period and then controlling the electrical conditions of some of the heating elements to cause a gradual decline in temperature for a predetermined period.

7. The method of operating an electrically heated furnace for annealing malleable iron castings which consists in causing material to progress through the annealing chamber within a predetermined time and during its progress controlling the electrical conditions in the heating elements, so that the temperature will first be raised at a rate substantially proportionate to the thermal conductivity of the material to a point above that at which the combined carbon begins to change into graphite, and then will be maintained at a substantially uniform temperature for a predetermined period and then will be gradually lowered to a point at which the desirable quantities of the material will not be injuriously affected by rapid cooling.

8. The method of operating an electrically heated furnace for annealing malleable iron castings, which consists in moving the material past the electrical heating elements and simultaneously controlling the movement of the material and the electrical conditions in the heating elements so that for a predetermined length of time, the material will be

exposed to heat sufficient to cause a rise in temperature at a rate substantially proportionate to the thermal conductivity of the material until a degree of temperature has been attained above that at which conversion of combined carbon into graphite begins, and thereafter controlling the electrical conditions of the heating elements during a predetermined portion of the travel of the material, so that the temperature of the material will be maintained for a predetermined time at a degree at which a predetermined amount of chemical change occurs, and thereafter cooling the material at a predetermined rate until the temperature has fallen below a point at which the desirable qualities of the material will be injuriously affected by rapid cooling.

9. In the art of producing malleable castings by an annealing process wherein the material is automatically subjected to heat treatment in a predetermined and definite cycle relative to temperature and time values, and wherein the heating of the treatment chamber is responsive to the activity of a control element individual to the specific nature of the material, the method of producing the control element which consists in subjecting a sample of the material to tests to ascertain the heat and time factors required to cause the desired chemical changes and then adapting the control element to cause the material to be subjected to predetermined temperature variations during predetermined periods of time.

10. The method of operating an electrically heated furnace for annealing malleable iron castings, which consists in subjecting a sample casting having the same formula as the castings to be annealed, to heat treatment in a device having a recording pyrometer indicating the heat conditions existing during the treatment, and upon the basis of data obtained from the treatment of the sample casting, preparing a controlling means adapted for use in the controlling mechanism for the annealing chamber whereby the electrical heating elements will be controlled in such a manner that castings exposed to the heat of the heating elements are first raised in temperature at a predetermined speed to a predetermined point, then maintained at that point during a predetermined period and thereafter permitted to cool at a predetermined rate of speed.

11. The method of annealing malleable castings which consists in ascertaining the conditions of temperature and time required during the annealing of a sample casting and thereafter subjecting other material of the same formula to similar heat treatment with the heat automatically controlled as to degree and duration to produce a predetermined progression of temperature values during a predetermined time.

12. The method of annealing malleable iron castings which consists in exposing the material to heat under conditions of control such that during a definite time cycle a progression of temperatures shall occur in the material corresponding to the thermal conductivity, temperature of conversion of combined carbon into graphite, and rate of

chemical change specific to the castings under treatment.

In testimony whereof I affix my signature in presence of two witnesses.

CHARLES T. HOLCROFT.

Witnesses:

HIRAM L. RITTS,  
KARL H. BUTLER.